

# United States Patent Office

3,359,131

Patented Dec. 19, 1967

1

3,359,131

## QUATERNIZED HALOMETHYL ETHERS

Robert J. Koshar, Lincoln Township, Washington County, and Harvey A. Brown, East Oakdale Township, Washington County, Minn., assignors to Minnesota Mining and Manufacturing Compay, St. Paul, Minn., a corporation of Delaware

No Drawing. Filed May 6, 1960, Ser. No. 27,279  
10 Claims. (Cl. 117—119.6)

This invention relates to halomethyl ethers and more particularly to certain new perfluoroalkyl-alkylene halomethyl ethers, to the quaternary ammonium salts prepared therefrom, and to a process for rendering textiles soil-resistant as well as oil and water repellent.

The novel halomethyl ethers of the invention contain a halomethyl group attached to a perfluoroalkyl group through an alkyleneoxy radical. The halomethyl ether group is quaternized by reaction with a tertiary nitrogenous organic base to form a quaternary ammonium salt, sometimes hereinafter referred to as a quaternized halomethyl ether. When the perfluoroalkyl group contains from about 4 to about 12 fully fluorinated carbon atoms, it has been found that the novel quaternary ammonium compounds of the invention can be employed as textile finishes to treat fibrous materials such as rayon, nylon, wool, silk, polyacrylate and polyacrylonitrile fibers and the like, and particularly to treat cellulosic materials such as cotton to produce a chemically bonded, soil-resistant, water- and oil-repellent finish thereon without thereby altering either color or tensile-strength.

While it has heretofore been found possible to produce valuable and useful soil-resistance, and oil- and water-repellency, in wool and certain synthetic fibers, it has been difficult to produce lasting effects on the cellulosic fibers. The finishes heretofore developed for this purpose, such as those which employ amido-quaternary amines as described in United States Patent No. 2,303,191, have been relatively easily removed, often by a single laundering operation. They have also required the deposit of relatively large amounts of the treating agent on the fibers, as compared with the compositions of the present invention.

It is an object of this invention to provide halomethyl ethers possessing fluorocarbon "tails" or residues.

Another object of this invention is to provide quaternary ammonium salts possessing fluorocarbon "tails."

Another object of this invention is to provide agents by means of which fibrous materials can be rendered oil- and water-repellent.

Another object of this invention is to provide agents by means of which cellulosic materials and particularly cotton fibers can be rendered lastingly oil- and water-repellent.

A further object of this invention is to provide oil- and water-repellent cellulosic materials such as cotton cloth.

Still another object of the invention is to provide a process for rendering cellulosic materials soil-resistant. Other objects will become apparent hereinafter.

In accordance with the above and other objects of this invention certain novel halomethyl ethers have been discovered which are useful for the production of quaternary ammonium salts containing a perfluorocarbon moiety, which may be designated as a fluorocarbon "tail" or residue. These compounds can be represented by the formula:



wherein  $R_f$  is a perfluoroalkyl group containing 4 to 12 carbon atoms, R is a divalent alkylene group selected from the group consisting of



and



2

wherein n is an integer from 1 to 10, m is an integer from 3 to 12 and X is chlorine or bromine.

The quaternary ammonium salts of the invention which are prepared from the above described halomethyl ethers, 5 can be represented by the formula:



wherein  $R_f$ , R, and X have the significance set forth hereinabove and Q is the radical of a tertiary nitrogenous base.

10 It is important that the perfluorocarbon "tail" or residue contain at least four carbon atoms, and the preferred number is six to ten. A terminal fluorocarbon chain of this minimum length is required in order to insolubilize and render the end of the molecule both hydrophobic and oleophobic.

15 The perfluorocarbon "tail" structure can include an oxygen atom linking together two perfluorinated carbon atoms, or a nitrogen atom linking together three perfluorinated carbon atoms, since these linkages are very 20 stable and do not impair the inert and stable fluorocarbon characteristic of the structure. The  $R_f$  radical can accordingly be a perfluoroalkyl group, a perfluorocycloalkyl group, or an oxygen-linked or nitrogen-linked perfluoroalkyl group.

25 The perfluorocarbon moiety of the molecule is inert and non-polar, and is both hydrophobic and oleophobic. It is repellent not only to oils but also to hydrocarbons. It imparts unique surface-active and surface-treating properties not possessed by corresponding compounds having 30 a hydrocarbon tail, the latter being oleophilic and highly soluble in oils and hydrocarbons and lacking the property of imparting soil-resistance which is a valuable feature of the compounds of this invention.

35 It will be evident that quaternization of the halomethyl ethers of the invention provides the quaternary ammonium salts of the invention which may thus also be referred to hereinafter as quaternized halomethyl ethers.

40 It has been found that the quaternized halomethyl ethers of the invention can be applied to woven and non-woven fabrics, as more fully described hereinafter, to provide oil- and water-repellency with improved resistance to laundering and dry cleaning.

45 The quaternized halomethyl ethers of the invention may be used as the sole component in the treating vehicle or as a component in a complex multi-ingredient formulation. For instance, excellent water and oil repellency and soil resistance is obtained on textile fabrics which are treated simultaneously with the quaternized halomethyl ethers of the invention and conventional finishes, such as 50 mildew preventatives, moth resisting agents, crease resistant resins, lubricants, softeners, sizes, flame retardants, anti-static agents, dye fixatives, and water repellents. In the treatment of paper the quaternized halomethyl ether may be present as an ingredient in a wax, starch, casein, 55 elastomer or wet strength resin formulation.

55 In addition to oil and water repellency and soil resistance properties, the quaternized compounds may be used to impart lower surface adhesion values and lower coefficients of friction to substrates. Accordingly, they 60 may also be used as mold release agents applied, for example, to wooden concrete forms, and related applications.

65 In the treatment of fabrics and fibrous materials, the quaternized halomethyl ethers of the invention may be employed in conjunction with other treating agents, such as crease resisting resins, sizes, softeners, and water repellents, by concurrent or sequential treatments. Known treating agents of these classes are as follows:

70 Crease resisting resins—

urea-formaldehyde resins, ethylene urea-formaldehyde resins, melamine-formaldehyde resins, tri-

azine-formaldehyde resins, epoxy resins, and poly-glycol acetals.

Sizes—

starch, casein, glue, polyvinyl alcohol, polyvinyl acetate, methyl cellulose, carboxymethyl cellulose.

Softeners—

polyethylene glycols, polyethylene, dimethyl polysiloxanes, amines and amides derived from fatty acids and ethylene oxide condensation products of such amines and amides.

Water repellents—

waxes, aluminum salts of fatty acids, silicone resins, chromium complexes of fatty acids, N-alkyl amidomethyl pyridinium salts, and melamine-formaldehyde resin condensates with amides from fatty acids.

The compounds of the invention are prepared by reaction of formaldehyde and hydrogen halide, e.g. hydrogen bromide or hydrogen chloride, with the corresponding fluorinated alcohol to produce a halomethyl ether, which is not necessarily isolated when quaternization is to be effected but is readily quaternized directly by addition of a tertiary amine such as pyridine. This procedure is conveniently carried out by passing the selected anhydrous hydrogen halide in gaseous form into a solution of the alcohol ( $R_fROH$ ) and paraformaldehyde in an inert solvent, such as toluene, benzene and the like until there is substantially no further absorption of the hydrogen halide. As the reaction is not strongly exothermic, no temperature control is required, although heating from about 25° C. to 100° C. (depending to an extent on the boiling point of the solvent used) may be resorted to, to insure completion of the reaction.

Another procedure which is very convenient since it avoids the use of halide is to react the alcohol and paraformaldehyde with the hydrohalide of the tertiary nitrogenous base, e.g. pyridine hydrochloride, in a suitable solvent such as the base. Isolation of the quaternary salt is then carried out as described above adding, if desired, a further amount of an organic solvent such as e.g. ether. The two procedures are to be considered equivalent.

The fluorinated alcohols of the invention are available by the procedure described in copending application Ser. No. 677,229. A perfluoroalkanesulfonyl chloride containing the desired  $R_f$  radical is added to a suitable derivative of a terminally unsaturated alcohol such as the acetate ester, the ester group merely serving as a temporary protective expedient for the hydroxyl group, in the presence of a free radical initiator, to form the corresponding omega-perfluoroalkyl-psi-chloroalkyl ester, which is hydrolyzed to produce the free alcohol. The latter compound is reduced if the chlorine atom is to be removed to produce the compounds of the invention in which  $R$  is  $-(CH_2)_m-$ . These reactions are represented diagrammatically:



wherein  $R_f$ ,  $m$  and  $n$  have the hereinabove set forth significance.

Suitable unsaturated alcohols for use in the process described, which are converted to their acetates by con-

ventional esterification procedures or may be used directly if desired, are:

- allyl alcohol
- 2-vinyl-ethanol
- 3-vinyl-propanol
- 6-vinyl-hexanol
- 9-vinyl-nonanol (i.e. undecenol)
- 10-vinyl-decanol
- 11-vinyl-undecanol
- 10. Perfluoroalkyl alcohols suitable for use in the invention include, for example, the following:
- 3-perfluorobutyl propanol-1
- 3-perfluoroctyl propanol-1
- 15 3-perfluorododecyl propanol-1
- 4-perfluoroctylbutanol-1
- 5-perfluorobutyl-pentanol-1
- 5-perfluoroctyl pentanol-1
- 5-perfluorododecyl pentanol-1
- 20 8-perfluorobutyl-octanol-1
- 8-perfluoroctyl-octanol-1
- 8-perfluorododecyl-octanol-1
- 11-perfluorobutyl-undecanol-1
- 11-perfluoroctyl-undecanol-1
- 25 11-perfluorododecyl-undecanol-1
- 11-(perfluoro-4-ethyl cyclohexyl)-undecanol-1
- 12-perfluoroctyl-dodecanol-1
- 13-perfluoroctyl-tridecanol-1

and the like.

Without isolation of the intermediate halomethylether, quaternization is effected in the inert solvent employed for the previous reaction after brief evaporation to remove excess hydrogen halide, or the reaction mixture may be further evaporated and some other solvent, such as anhydrous ether or dioxane, in which the quaternary salt is insoluble, may be added. The desired tertiary organic base or amine is then added in the stoichiometric amount while maintaining the reaction mixture at a temperature in the range of about 25° C. to about 100° C. Any tertiary nitrogenous organic base which is capable of forming a salt or quaternary compound is suitable for this purpose, including, for example, trialkyl amines such as trimethylamine, tributylamine and triododecylamines; cycloalkyl amines such as tricyclohexylamine; aralkyl amines such as benzyl dimethylamine; arylamines such as dimethylaniline; and heterocyclic amines such as pyridine, picoline, lutidine, quinoline and the like. Pyridine is particularly preferred for convenience and economy in the formation of cloth-treating agents as shown above.

Illustrative of the quaternized halomethylethers of the invention are the following:

- 3-(perfluorobutyl)propanoxymethyl trimethyl ammonium bromide
- 55 3-(perfluoroctyl)-propanoxymethyl phenyl dimethyl ammonium chloride
- 3-(perfluorododecyl)-propanoxymethyl tricyclohexyl ammonium chloride
- 4-(perfluoroctyl)-butanoxymethyl tributyl ammonium bromide
- 5-(perfluorobutyl)-pentanoxymethyl pyridinium chloride
- 5-(perfluoroctyl)-pentanoxymethyl triethyl ammonium bromide
- 5-(perfluorododecyl)-pentanoxymethyl pyridinium chloride
- 8-(perfluorobutyl)-octanoxymethyl quinolinium chloride
- 8-(perfluoroctyl)-octanoxymethyl picolinium chloride
- 8-(perfluorododecyl)-octanoxymethyl benzyl dimethyl ammonium chloride
- 70 11-(perfluorobutyl)-undecanoxymethyl pyridinium chloride
- 11-(perfluoroctyl)-undecanoxymethyl pyridinium chloride
- 11 - (perfluorododecyl) - undecanoxymethyl pyridinium chloride

- 11-(perfluoro-4-ethyl-cyclohexyl)-undecanoxymethyl trimethyl ammonium chloride  
 12-(perfluoroctyl)-dodecanoxymethyl tributyl ammonium chloride  
 13-(perfluoroctyl)-tridecanoxymethyl pyridinium bromide

and the like.

The quaternized compounds of the invention are employed for treating woven or non-woven fibrous materials including wool, cotton, rayon, acetate, nylon and the like textiles, or paper, leather, wood, felt and similar organic fibrous constructions, and particularly cellulosic materials, by applying the selected quaternary ammonium derivatives, in aqueous medium buffered to about pH 6, to the cloth, removing any excess, drying at a temperature in the range of about 40° to 100° C., and heating the dried material to about 100° to 140° C. for a period of the order of about 5 to 30 minutes to fix the finish. Thereafter the material is desirably washed in a mildly alkaline aqueous solution to remove any residual acidic material, and dried. The treatment may be followed by a single aqueous wash before drying, if desired, although this may be omitted since subsequent laundering of the treated fabric accomplishes the same purpose. This treatment may be termed a finishing treatment, since it is most usefully applied after weaving, forming, dyeing, weighting, filling or the like have been carried out. Cotton cloth so treated contains residual fluorine, as indicated by standard analytical methods, indicating that at least a portion of the treating agent is retained and has probably reacted in some fashion, probably through the hydroxyl groups present in the fiber, although this hypothesis clearly is not to be construed as limiting the invention.

It is a surprising feature of cotton fabric treated with these quaternary derivatives that not only is the cloth rendered oil- and water-repellent but also it possesses a considerable degree of soil resistance, that is, it does not become soiled as readily as untreated fabric. Furthermore, when soiled the fabrics thus treated are readily launderable or dry-cleaned to a clean state, after which they retain their oil- and water-repellency. The value of cloth so treated, for example, for children's clothes, or for uniforms for workers around oily machinery, automotive service men and the like will be readily apparent.

The color of the fabrics treated with the compositions of the invention, and their tensile strength, are not affected by the treatment. The hand of cotton fabrics appears to be improved by the treatment.

It is noted that the finishing treatment of the invention can be applied to resin-treated, wrinkle-resistant fabrics without adversely affecting the desirable non-wrinkling feature of such fabrics.

The procedure for the preparation of the quaternized compounds of the invention, and the application of the latter to fabrics, especially cellulosic materials are more specifically illustrated in the following examples, in which all parts are by weight and all percentages of solutions w./v. unless otherwise specified. It will be understood that these examples are illustrative only to show the best mode presently contemplated of practicing the invention and are not to be construed as limiting as to the scope of the invention.

#### Example 1

The following procedure is used to prepare 5-perfluorooctyl-pentanol-1.

A mixture of 26.8 g. (0.052 mole) of perfluoroctane sulfonyl chloride and 5.0 g. (0.050 mole) of 4-pentenoic acid (allyl-acetic acid) is heated for four hours at about 120-145° C. in the presence of a catalytic amount (1.0 g.) of di-tertiary butyl peroxide. The reaction mixture is fractionally distilled under reduced pressure and the fraction boiling at about 100° C. at 0.01 mm. is collected. After recrystallization from a mixture of chloroform and

carbon bisulfide, the 4-chloro-5-(perfluoroctyl)-pentanoic acid thus prepared melts at about 89-90° C.

The 4-chloro-5-(perfluoroctyl)-pentanoic acid thus prepared is hydrogenated by shaking a solution of 8.00 g. (0.0145 mole) of the acid and 2.5 g. (0.062 mole) of sodium hydroxide in a mixture of 30 ml. of water and 30 ml. ethanol for 3 hours at 140° C. in a rocking high-pressure hydrogenation apparatus, in the presence of 4 g. of Raney nickel catalyst and with hydrogen supplied at 2500 p.s.i. pressure. After removal of the catalyst and evaporation to dryness, an amorphous residue is obtained comprising sodium 5-(perfluoroctyl)-pentanoate. By dissolving this residue in water followed by acidification of the resulting solution, the saturated perfluoroalkyl aliphatic acid formed by hydrogenation is recovered as a waxy white solid, which can be distilled at 100° C. at 0.02 mm. pressure. After recrystallization from carbon bisulfide, the 5-(perfluoroctyl)-pentanoic acid thus prepared melts at about 86.5-87.3° C. The procedure described in U.S. Patent 2,666,797, using lithium aluminum hydride, is employed for reduction of the acids to the corresponding alcohols. A suspension in ether of 30 parts of 5-(perfluoroctyl) pentanoic acid is added to a solution of 3 parts of lithium aluminum hydride in about 200 parts of anhydrous ether. The reaction mixture is stirred for about 48 hours and then is treated with water and neutralized with sulfuric acid. The reaction mixture is extracted several times with ether, and the ether extracts are combined, dried and fractionally distilled in vacuo. There is obtained 5-(perfluoroctyl)-pentanol boiling at about 108° C. at 2.5 mm. pressure of mercury.

A mixture of 25 parts (0.05 mole) of 5-perfluoroctyl-pentanol-1 and 1.5 parts (0.5 mole) of paraformaldehyde in about 85 parts of benzene is warmed to effect solution and anhydrous hydrogen chloride gas is passed into the warm solution until there is no further absorption. This requires about 1.5 hours. The solution is evaporated under reduced pressure to remove excess hydrogen chloride and benzene and 3.9 parts (0.05 mole) of anhydrous pyridine is added to the residue. The resultant mixture is warmed whereupon it solidifies with the formation of 5-(perfluoroctyl)-pentoxymethyl pyridinium chloride which is suspended in ether, collected, washed further with ether and dried.

Calculated for



N, 2.21%; Found: N, 2.20%.

#### Example 2

10-chloro-11-perfluoroctylundecyl acetate is prepared as follows: A 3-necked flask containing a glass encased magnetic stirring bar and fitted with a thermometer, two addition funnels and water cooled reflux condenser and a subsequent liquid air trap is charged with 30 parts of perfluoroctanesulfonyl chloride, 12 parts undecenyl acetate and 2 parts of di-tertiary butyl peroxide. In one addition funnel is placed 49.5 parts of undecenyl acetate and in the other 120 parts of perfluoroctanesulfonyl chloride containing a further 2 parts of di-tertiary butyl peroxide. The flask is heated to about 120° C. over about 40 minutes when the reaction commences exothermically and further additions of reactions are made gradually during about a further 30 minutes. The reaction mixture is maintained at about 130° C. for about 1 hour longer during which time 15 parts of sulfur dioxide are collected in the liquid-air-trap. The reaction mixture is distilled under reduced pressure. 10-chloro-11-perfluoroctylundecyl acetate distills at about 170° C. at 1.5 mm. Hg as a liquid which solidifies to a white solid at room temperature.

Reduction of 65 parts of 10-chloro-11-perfluoroctylundecyl acetate in 25 parts of triethylamine with hydrogen at about 2500 p.s.i. and about 140° C. for about 2.5

hours in the presence of 3 parts of Raney nickel (previously washed with triethylamine) provides a solution of 11-perfluoroctyl-undecyl acetate which is recovered as an oil by filtration and evaporation. Saponification of the oil in 80 percent aqueous ethanol using potassium hydroxide in excess provides 11-perfluoroctylundecanol as a rather viscous oily liquid boiling at about 120° to 124° C. at about 0.2 mm. Hg which solidifies on standing.

The halomethylation procedure of Example 1 is repeated using benzene as a solvent and the intermediate 11-perfluoroctylundecanoxymethyl chloride is recovered, taken up in anhydrous ether and reacted with pyridine. 11-perfluoroctylundecanoxymethyl pyridinium chloride is obtained as white crystals melting at about 78° C. and decomposing at about 150° C. on further heating.

Calculated: N, 1.95%. Found: N, 1.99%.

The procedure is repeated employing triethylamine in place of pyridine and rather impure 11-perfluoroctylundecanoxymethyl triethyl ammonium chloride is obtained melting from about 85° C. upward and decomposing at about 120° C.

Calculated: N, 1.90%; C, 42.4%; F, 43.6%. Found: N, 2.04%; C, 42.4%; F, 38.1%.

By the same procedure the quinolinium salt is prepared using quinoline in place of pyridine. 11-perfluoroctylundecanoxymethyl quinolinium chloride melts at about 120° to 125° C.

Calculated: C, 45.5%; N, 1.83%; F, 42.1%. Found: C, 46.2%; N, 2.08%; F, 39.0%.

The procedure is repeated using anhydrous hydrogen bromide in place of hydrogen chloride to form 11-perfluoroctylundecanoxymethyl bromide which is then reacted with pyridine as above. The resultant 11-perfluoroctylundecanoxymethyl pyridinium bromide monohydrate softens at about 90° C. and decomposes above about 175° C.

Calculated (for monohydrate): C, 39.4%; N, 1.84%; Br, 10.5%. Found: C, 39.2%; N, 2.3%; Br, 13.7%.

In the same way as described hereinabove for the preparation of 5-perfluoroctyl pentanol, using 10-undecanoic acid in preparation of the perfluoro acid instead of allyl-acetic acid, there is produced 11-(perfluoroctyl)-undecanoic acid, which on reduction yields 11-(perfluoroctyl)-undecanol boiling at about 122-126° C. at 0.10-0.15 mm. pressure of mercury and melting at about 69° to 71° C.

A mixture of 40 parts of 11-perfluoroctylundecanol and 6 parts of paraformaldehyde in 150 parts of pyridine is refluxed at 100° C. for about 1 hour and sulfur dioxide is passed into the solution at 90° to 100° C. for about 3/4 hour. The solution is allowed to stand overnight and excess pyridine is evaporated under reduced pressure. The residue is extracted twice with ether to remove unreacted alcohol. The remainder is dissolved in 100 parts of benzene and the mixture evaporated and dried at 70° C. and 10 mm. Hg pressure for 1.5 hours. The tacky residue comprising 11-perfluoroctylundecanoxymethyl pyridinium sulfite is insoluble in ether or acetone but dissolves in water giving a foamy solution.

Analysis shows the presence of S, 10.3%, and N, 4.8%.

### Example 3

By the procedure described above, 64.1 parts of perfluoromethanesulfonyl chloride and 81 parts of 10-undecenyl acetate are reacted at 130° to 148° C. for 5 1/2 hours in the presence of 4 parts of benzoyl peroxide in a pressure vessel and the product, 10-chloro-11-perfluoromethyl-undecyl acetate, is isolated by fractional distillation as a colorless liquid, boiling from about 120° to 123° C. at about 0.8 mm. Mg pressure and having  $n_D^{25}=1.4240$ .

Calculated for  $C_{14}F_3H_{24}ClO_2$ : C, 53.2%; F, 18.0%. Found: C, 53.4%; F, 18.0%.

A mixture of 56.2 parts of 10-chloro-11-perfluoromethyl undecyl acetate and 3 parts of Raney nickel catalyst (washed with triethylamine) in 50 parts of triethyl-

amine is heated at about 145° to 175° C. under about 2000 to 2500 p.s.i. of H<sub>2</sub> pressure for 5.5 hours and then cooled and filtered. The solution is evaporated to give a liquid residue. This liquid (48 parts) is refluxed for 15 hours with stirring in 100 parts of ethanol containing 17 parts of potassium hydroxide in 40 parts of water. The saponification mixture is evaporated to remove alcohol, diluted with thrice its volume of water, acidified and thoroughly extracted with ether. The ethereal solution is evaporated under reduced pressure to provide crude 11-perfluoro-methyl-undecanol which is conveniently freed from unsaturated materials resulting from incomplete reduction by catalytic hydrogenation.

A total of 48 parts of crude 11-perfluoromethyl-undecanol containing some of the corresponding  $\Delta^{10}$  unsaturated compound is shaken with 5 parts of Raney-nickel catalyst in 51 parts of triethylamine and 35 parts of ethanol at about 150° C. for 2 hours. The filtered reaction mixture is evaporated to dryness and fractionally distilled. 11-perfluoromethyl-undecanol boils at about 107° to 109° C. at about 1.5 mm. Hg. pressure and melts at about 33° C.

Calculated for  $C_{12}F_3H_{23}O$ : F, 23.7%; C, 60.0%. Found: F, 22.5%; C, 60.2%.

A mixture of 30 parts of 11-perfluoromethyl-undecanol and 4 parts of paraformaldehyde in about 85 parts of toluene is saturated with anhydrous hydrogen chloride for about 1 hour until the solution becomes clear. The toluene is removed under vacuum (below 1 mm. Hg) at 40° C. The residue is taken up in 100 parts of ether and filtered and 15 parts of pyridine added to the filtrate. The resultant solution is refluxed for 1 hour and the precipitate collected. It is 11-perfluoromethyl-undecanoxymethyl-pyridinium chloride melting at about 80° C.

Calculated for  $C_{18}F_9H_{29}NOCl \cdot \frac{1}{3}H_2O$ : N, 3.75%; F, 15.3%; H<sub>2</sub>O, 1.6%. Found: N, 3.7%; F, 14.0%; H<sub>2</sub>O, 1.4%.

The process for production of soil-resistant, water- and oil-repellent cloth using the quaternary derivatives of the compounds of this invention is carried out as follows:

The treating solution is prepared by warming sodium acetate trihydrate and the selected treating agent in water at the desired concentrations, which can range from about 0.1 to about 5 percent, at about 30° to 40° C. until solution is effected. It is to be noted that at higher concentration the solution tends to become mucilaginous, resembling a colloidal dispersion. The cloth to be treated is soaked in the solution for 1 minute, removed and squeezed so that a weight of solution approximately equal to 75 to 125 percent of the weight of the cloth is retained. Under these conditions, the preferred concentration of treating solution ranges from about 0.5 to about 2 percent. The cloth is then dried for about 10 to 30 minutes at 40° to 100° C. and the treatment is fixed by heating the cloth for about 5 to 30 minutes at from about 100° to 140° C. The fixed, treated cloth is washed for about 30 minutes in an aqueous solution containing 0.1 percent w/v. of sodium lauryl sulfate and 0.2 percent w/v. sodium carbonate, at about 50° to 60° C., rinsed thoroughly and again dried. Other alkaline agents, such as dilute alkali metal hydroxides, bicarbonates, ammonium hydroxide and the like can be used instead of alkali metal carbonates, to produce a mildly alkaline aqueous washing solution.

The effectiveness of the treatments is determined by means of tests for spray rating, oil repellency rating and visual estimation of soil repellency both before further treatment and after one or more cycles of laundering and/or dry cleaning.

For test purposes, laundering is accomplished by washing in an automatic washing machine of the stationary tub type using a detergent under normal household procedures or by means of a standard 60 minute cycle in a Launder-O-Meter, using chip soap as specified in ASTM D-496. Dry-cleaning is performed by available com-

mercial procedures employing, for example, perchloroethylene or naphtha.

Determination of water repellency rating is by means of the "Spray Test" (Standard Test Method No. 22-52, published in the 1952 Technical Manual and Yearbook of the American Association of Textile Chemists and Colorists, vol. XXVIII, p. 136).

Oil repellency of the treated cloth is measured by a severe test in which its resistance to penetration by solutions of mineral oil in heptane is determined. (Higher proportions of heptane bring about quicker penetration.) A material wet by mineral oil alone in less than 3 minutes rates zero, if it is only wet after 3 minutes it rates fifty, while resistance to penetration by a mixture of equal volumes of heptane and mineral oil rates 100. The ratings for resistance for 3 minutes are as follows:

| Percent heptane: | Rating |
|------------------|--------|
| 0                | 50     |
| 20               | 70     |
| 30               | 80     |
| 40               | 90     |
| 50               | 100    |
| 60               | 100+   |

A rating of 70 or higher indicates a high degree of resistance to staining by salad oil and the like.

Dry soil resistance simulates soil repellency of a material under especially exaggerated conditions. A control sample of untreated cloth and the treated sample to be tested are shaken together in a paper bag with about 2 ounces of a standard synthetic soil mixture (having the composition described in the report of Salsbury, et al., American Dyestuff Reporter, Mar. 26, 1956, p. 199), then removed and sharply struck against a solid object to remove loosely adherent soil and compared visually with a similarly soiled untreated sample. The ratings are from 0 to 3. These correspond to visual estimation to:

- 0 as dark as control (untreated cloth sample)
- 1 slightly less dark than control
- 2 more than about half as dark as control
- 3 less than about half as dark as control

While the ratings are to some extent subjective, and may vary to a certain extent as to the degree of soil involved, it is significant that there is markedly less soiling of samples treated with the compounds of the invention and this property is retained after laundering.

The synthetic soil mixture is prepared by blending the following:

|                                                            | Parts by wt. |
|------------------------------------------------------------|--------------|
| Peat moss                                                  | 38           |
| Portland cement                                            | 17.0         |
| Kaolin clay                                                | 17.0         |
| Silica (800 mesh)                                          | 17.0         |
| Furnace black (high leading, blue tone, powdered, Malacco) | 1.75         |
| Red iron oxide                                             | 0.5          |
| Mineral oil (heavy)                                        | 8.75         |

The blend is placed in a large pan and dried in a forced draft convection oven for 2 hours at 50° C. and then ground in a ball mill. The finely divided material which is produced is stored in a desiccator over calcium chloride or sulfuric acid.

The following example further illustrates the treatment of cloth by the process of and using the compounds of the invention.

#### Example 4

Treating solutions are prepared as described above by warming 1 part of sodium acetate trihydrate and two parts of each of the following quaternized compounds of Example 2 in 100 parts of water. These are designated by the letters shown.

(A) 11-perfluoroctylhendecaneoxymethyl pyridinium chloride

- (B) 11-perfluoroctylhendecaneoxymethyl pyridinium bromide
- (C) 11-perfluoroctylhendecaneoxymethyl triethylammonium chloride
- (D) 11-perfluoroctylhendecaneoxymethyl quinolinium chloride

Samples of cotton jeans cloth are treated with the respective solutions, dried at 100° C. for 30 minutes, heated for 5 minutes at 135° C. (A, D and D), or 121° C. (B), washed and dried as described above, and rated as follows:

|           | Oil | Spray | Percent F |
|-----------|-----|-------|-----------|
| 15 A----- | 80  | 90    | 0.9       |
| B-----    | 100 | 70    | 0.5       |
| C-----    | 50+ | 80    | 0.23      |
| D-----    | 70  | 80    | (*)       |

\*Not determined.

- 20 All show appreciable soil resistance and retain an appreciable percentage of oil- and water-repellency after laundering or dry-cleaning. Substantially the same results are observed when nylon and woolen fabrics are similarly treated.
- 25 The 11-perfluoromethylhendecanoxyethyl pyridinium chloride of Example 3 above is applied similarly to cotton cloth and is found to exert no appreciable repellent effect. The perfluoro alkyl group must contain more than one carbon atom and preferably has four or more perfluorinated carbon atoms.

The procedure of Example 1 is repeated employing 1,1-dihydro-perfluoroctanol and the starting compound is recovered unchanged; there is no reaction when  $n$  of the divalent alkylene group is as low as 1. It is found that  $n$  should be from 3 to 12.

- 30 3-(perfluoropropyl)-propanol is prepared starting with ethyl perfluorobutyrate as follows: Approximately equimolar quantities of ethyl perfluorobutyrate, methyl acetate and sodium methoxide are used. The ethyl perfluorobutyrate is added to a cooled solution of sodium methoxide in absolute ether, with continued cooling. After stirring this mixture for approximately two hours the methyl acetate is added, whereupon a clear solution forms. The solution is stirred for approximately 16 hours and then fractionally distilled under reduced pressure, to remove solvents and to obtain methyl 3-(perfluoropropyl)-3-keto propionate as the main product. The keto-ester thus obtained is hydrogenated under pressure with Raney nickel catalyst, in ether solution, under the usual conditions, for about two hours. The catalyst is removed by filtration and the filtrate is fractionally distilled in vacuo, whereupon methyl 3-(perfluoropropyl)-3-hydroxy propionate is recovered, boiling at about 85° C. at 15 mm. pressure and having refractive index  $n_D^{25}=1.3513$ .
- 35 About 157 parts of the hydroxy ester thus obtained and 175 parts of phosphorous pentoxide are mixed and allowed to stand for approximately 16 hours (a rather mixing). The reaction mixture is then filtered and the filtrate is purified by fractional distillation. There is obtained methyl 3-(perfluoropropyl) acrylate which boils at 121-124° C. at 732 mm. pressure and has refractive index  $n_D^{25}=1.3362$ . The acrylic ester is hydrogenated in ether solution using Raney nickel catalyst and high pressure under the usual conditions. The reaction mixture is filtered and the filtrate is fractionally distilled under reduced pressure. There is obtained the corresponding saturated ester, methyl 3-(perfluoropropyl)propionate, which boils at 42° C. at 12 mm. pressure and has refractive index  $n_D^{25}=1.3276$ . To a solution of 7.6 g. (.2 mole) of lithium aluminum hydride in 500 ml. of ether are added 49 g. (0.191 mole) of the methyl 3-(heptafluoropropyl)-propionate dissolved in 100 ml. of ether, at such a rate that vigorous refluxing is maintained. The mixture is then stirred for 1 hour and an excess of methanol is added to hydrolyze the complex. The reaction mixture

is next acidified with dilute sulfuric acid. The ether layer is separated and the aqueous layer is further extracted with about an equal volume of ether. The combined ether phases are evaporated to remove the ether and the residue is fractionally distilled. The 3-(heptafluoropropyl)-propanol thus obtained boils at about 140-141° C. at 745 mm. pressure and has index of refraction,  $n_D^{24}$ =1.3270.

By repeating the procedure of Example 1, employing perfluoro-n-butanesulfonyl chloride, perfluoro-4-ethylcyclohexanesulfonyl chloride, and perfluorododecane sulfonyl chloride (prepared by the process of Brice et al. as disclosed in U.S. Patent No. 2,732,398) instead of perfluoroctanesulfonyl chloride, there are obtained, respectively, 5-(perfluorobutyl)-pentanoic acid, perfluoro-4-ethylcyclohexyl pentanoic acid and 5-(perfluorododecyl)-pentanoic acid. Upon reduction, these acids yield the corresponding 5-(perfluoropentyl)-pentanol, 5-(perfluoro-4-ethylcyclohexyl)-pentanol and 5-(perfluorododecyl)-pentanol, respectively.

When 3 - perfluoropropyl-propanol, 5 - perfluorobutyl-pentanol, 5-perfluoro(4-ethyl cyclohexyl)-pentanol and 5-perfluorododecyl-pentanol are converted to the respective corresponding halomethyl ethers and quaternized by the procedure of Example 1, using pyridine, the respective crystalline quaternary chlorides are isolated, viz: 3-(heptafluoropropyl)propanoxymethyl pyridinium chloride, 5-nonafluorobutyl)-pentanoxymethyl pyridinium chloride, 5-perfluoro(4-ethyl cyclohexyl)pentanoxymethyl pyridinium chloride and 5-perfluorododecyl)-pentanoxymethyl pyridinium chloride. When each of these is made up into a treating solution at 2 percent concentration with sodium acetate, applied to cotton cloth as described above, and tested for oil- and water-repellency, it is found that all except the 3-heptafluoropropylpropanoxymethyl pyridinium chloride provide significant oil- and water-repellency. The latter compound does not produce this effect, showing that the perfluoroalkyl group must contain 4 or more carbon atoms.

The solutions used for treating fabrics as set forth above can also be applied to paper with slight modification in procedure to avoid damaging the structure of the paper, which, as is well known, is weakened by treatment with water. Thus, the excess of treating solution is removed by permitting the paper to drip dry or by running the web between rolls, while drying and fixing are accomplished by heating the individual sheets or by hot-roll calendering long strips or continuous rolls. The treated paper is oil- and water-repellent. Wooden surfaces are rendered oil- and water-repellent by applying the solution as a paint, drying and heating as above followed by a mildly alkaline wash and drying again.

#### Example 5

When the solution designated A in Example 4 above is made up to contain additionally 10 percent of a melamineformaldehyde condensate (of the type employed for producing crease resistance) and 1 percent of an accelerator for the cure thereof and cotton cloth is treated with this solution and cured following the procedure described above, it is found that the washed and dried cloth shows crease-resistance and is oil- and water-repellent. Substantially similar results are obtained when cloth initially treated with a crease-resistance promoting resin is subsequently treated with solution A above.

What is claimed is:

1. A compound of the formula



wherein  $R_f$  is perfluoroalkyl having 4 to 12 carbon atoms,  $Q$  is a tertiary nitrogenous organic residue selected from the group consisting of trialkylamino having 3 to about 36 carbon atoms, tricyclohexylamino, aralkyl amino having about 8 carbon atoms, aryl amino having about 8 carbon atoms, pyridino, picolino, lutidino and quinolino,  $X$  is a halogen of the group consisting of chlorine and

bromine and  $R$  is a divalent radical selected from the group consisting of:



and



wherein  $n$  is an integer from 1 to 10 and  $m$  is an integer from 3 to 12.

2. A compound of the formula:



wherein  $R_f$  is perfluoroalkyl having 4 to 12 carbon atoms,  $X$  is a halogen of the group consisting of chlorine and bromine, and  $R$  is a divalent radical selected from the group consisting of:



and



wherein  $n$  is an integer from 1 to 10 and  $m$  is an integer from 3 to 12.

3. A compound of the formula:



wherein  $R_f$  is perfluoroalkyl of 4 to 10 carbon atoms,  $Q$  is a tertiary nitrogenous organic residue selected from the group consisting of pyridino, picolino, lutidino, quinolino and dimethylanilino,  $X$  is a halogen selected from the group consisting of chlorine and bromine and  $R$  is a divalent radical selected from the group consisting of:



and



wherein  $n$  is an integer from 1 to 7 and  $m$  is an integer from 3 to 9.

4. A compound of the formula



wherein  $R_f$  is perfluoroalkyl of 4 to 10 carbon atoms,  $X$  is halogen selected from the group consisting of chlorine and bromine, and  $R$  is a divalent radical selected from the group consisting of:



and



wherein  $n$  is an integer from 1 to 7 and  $m$  is an integer from 3 to 9.

5. 5-perfluoroctylpentylloxymethyl pyridinium chloride.

6. Omega-perfluoroctyl-undecanoxymethyl pyridinium chloride.

7. A compound of the formula



wherein  $R_f$  is perfluoroalkyl having 4 to 12 carbon atoms,  $X$  is halogen of the group consisting of chlorine and bromine and  $m$  is an integer from 3 to 12.

8. The process for rendering fibrous materials water- and oil-repellent, which comprises treating the fibrous material with a compound of the formula:



wherein  $R_f$  is perfluoroalkyl having 4 to 12 carbon atoms,  $Q$  is a tertiary nitrogenous organic residue selected from the group consisting of trialkylamino having 3 to about

36 carbon atoms, tricyclohexylamino, aralkyl amino having about 8 carbon atoms, aryl amino having about 8 carbon atoms, pyridino, picolino, lutidino and quinolino,

$X$  is a halogen of the group consisting of chlorine and bromine and  $R$  is a divalent radical selected from the group consisting of:



and



wherein  $n$  is an integer from 1 to 10 and  $m$  is an integer from 3 to 12; in aqueous medium buffered to about pH 5.5 to 6.5, drying the treated fibrous material and heating the dried, treated material to a temperature in the range of about 100° to 140° C. for a period of about 5 to 30 minutes.

9. A fabric finished with a compound of the formula:



wherein  $R_f$  is perfluoroalkyl having 4 to 12 carbon atoms,  $Q$  is a tertiary nitrogenous organic residue selected from the group consisting of trialkylamino having 3 to about 36 carbon atoms, tricyclohexylamino, aralkyl amino having about 8 carbon atoms, aryl amino having about 8 carbon atoms, pyridino, picolino, lutidino and quinolino,  $X$  is a halogen of the group consisting of chlorine and bromine, and  $R$  is a divalent radical selected from the group consisting of:



and



wherein  $n$  is an integer from 1 to 10 and  $m$  is an integer from 3 to 12, whereby the fabric contains residual combined fluorine and has oil- and water-repellent properties.

10. A cellulosic fabric having oil- and water-repellent

5

properties, finished with 11-perfluorooctane-hendecanoxy-methyl pyridinium chloride.

#### References Cited

#### UNITED STATES PATENTS

|           |         |                    |           |
|-----------|---------|--------------------|-----------|
| 2,727,923 | 12/1955 | Husted -----       | 260—567.6 |
| 2,767,189 | 10/1956 | Erickson -----     | 260—567.6 |
| 2,804,402 | 8/1957  | Williams -----     | 117—139.4 |
| 2,812,350 | 11/1957 | Niederhauser ----- | 260—567.6 |
| 2,913,500 | 11/1959 | Becke et al. ----- | 260—614   |
| 2,915,524 | 12/1959 | Truitt -----       | 260—297   |

#### OTHER REFERENCES

- 15 Knunyants et al.: Chem. Abstracts, vol. 43, col. 6163 (1949).  
 Brey et al.: J. Am. Chem. Soc., vol. 79, pp. 6533—6 (1957).  
 Park et al.: Chem. Abstracts, vol. 53, col. 6058 (1959).  
 20 Jarvis et al.: J. Phys. Chem., vol. 63, pp. 727—734 (1959).  
 JOHN D. RANDOLPH, *Primary Examiner.*  
 D. T. McCUTCHEON, I. MARCUS, *Examiners.*  
 25 R. T. BOND, *Assistant Examiner.*

UNITED STATES PATENT OFFICE  
CERTIFICATE OF CORRECTION

Patent No. 3,359,131

December 19, 1967

Robert J. Koshar et al.

It is hereby certified that error appears in the above numbered patent requiring correction and that the said Letters Patent should read as corrected below.

Column 5, line 11, for "actate" read -- acetate --; column 10, lines 57 and 58, for "(a rather mixing)" read -- (a rather strong exothermic reaction being noted shortly after mixing) --; column 11, line 27, for "5-nonafluorobutyl)" read -- 5-(nonafluorobutyl) --.

Signed and sealed this 14th day of January 1969.

(SEAL)

Attest:

Edward M. Fletcher, Jr.

Attesting Officer

EDWARD J. BRENNER

Commissioner of Patents